

## UNITED STATES PATENT OFFICE.

CARL D. PRATT, OF TAMAQUA, PENNSYLVANIA, ASSIGNOR TO ATLAS POWDER COMPANY, OF WILMINGTON, DELAWARE, A CORPORATION OF DELAWARE.

## BLASTING-POWDER COMPOSITION.

No Drawing.

Application filed May 31, 1924. Serial No. 717,141.

To all whom it may concern:

Be it known that CARL D. PRATT, citizen of the United States, residing at Tamaqua, in the county of Schuylkill and State of Pennsylvania, has invented certain new and useful Improvements in Blasting-Powder Compositions, of which the following is a specification.

My invention relates to improvements in blasting powder compositions and it has for its object to provide a new and highly useful commercial blasting explosive which will possess characteristics of safety far beyond those of ordinary black blasting powder.

The record of the Bureau of Mines of the United States, covering the period from 1908 to 1923 shows that seventy-one coal mine explosions have been caused directly by the use of black blasting powder or by black blasting powder and dynamite, killing more than eight hundred men, injuring many others and causing untold property damage. This serious situation can be largely corrected by the substitution for black blasting powder, of what are known as "permissible" explosives, that is, explosives which have passed certain tests prescribed by the Bureau of Mines. Tests conducted by said bureau, and verified in actual coal mining operations, have demonstrated conclusively that a permissible explosive has a very much shorter and cooler flame than black blasting powder and a very much cooler flame than other high explosives.

With the foregoing facts in mind it has been my aim to provide a series of blasting powder compositions, which have decreased tendencies, compared with current commercial grades of blasting powder compositions, to ignite inflammable gases and dusts, or mixtures thereof; as for example, those occurring in coal-mines.

It should be expressly understood that my invention is not concerned with so-called "high explosives", but is concerned entirely with the type of so-called "low explosives", herein referred to as "blasting powders."

"High explosives" include both individual compounds and mixtures of ingredients, which are able to suddenly decompose in the manner of a detonation, through almost instantaneous disintegrations and reactions, as influenced by heat or shock or both. "Low explosives," on the other hand, consist only of mixtures of ingredients, of such a nature as to react with each other, in the form of a rapid combustion, as distinguished from a sudden disintegration, when influenced by heat. It is a peculiarity of "high explosives" that they decompose with a much higher speed than "low explosives", thus exerting quicker and more disruptive actions than the slower and consequently more propulsive "low explosives."

My improved blasting powders may, properly, be referred to as "safety blasting powders," since they are safer for use under gaseous and dusty conditions, such as coal-mining, than the current blasting powders, just as permissible high explosives are safer for use in coal-mines than straight nitroglycerine dynamites or gelatins.

As a result of a very exhaustive study of many principles and extensive experimentation in following out these principles in a very large number of mixtures, I have been able to devise a series of blasting powders, with decreased tendencies (compared with current commercial blasting powders) to ignite inflammable gases and dusts or mixtures thereof, through the discovery that carbohydrates together with tartrates and oxalates, when added to blasting powder compositions, consisting of one or more metallic nitrates, sulphur and one or more materials that are essentially carbon, will effectively produce these improvements in combination or singly.

Carbohydrates, I have found, such as sugar, cellulose, glucose, starch and the like, produce the desired decreased tendencies to ignite inflammable gases and dusts or mixtures thereof, through their introduction into the chemical constitutions of blasting powders, of greater amounts of carbon and

hydrogen in proportion with oxygen, to the extent of markedly decreasing the amounts of heat evolved by the decomposition reactions of such compositions.

- 5 I have also found that tartrates and oxalates, such as sodium potassium tartrate, ammonium oxalate and the like, produce the desired decreased tendencies to ignite inflammable gases and dusts or mixtures thereof, when in intimate contact with the decomposition reactions of blasting powder compositions, especially those including one or more carbohydrates, through their heat absorbing abilities.
- 10 15 Further, I have discovered that blasting powder compositions, including carbohydrates, together with tartrates and oxalates, selected in combination, or singly, to suit requirements, together with the usual blasting powder ingredients (metallic nitrates, sulphur and materials that are essentially carbon), will actually have several times less tendency to ignite inflammable gases and dusts or mixtures thereof, than the 20 current commercial grades of blasting powders. That is, charges of my "safety blasting powders" (hereinbefore defined) that I am able to fire into certain gases and dusts or mixtures thereof, without igniting them, 25 are several times the weight of current commercial blasting powder charges which will ignite the same gases and dusts or mixtures thereof, under like conditions.

It should be expressly understood that the 30 scope of my invention is broad enough to include any manner of introduction of the cooling ingredients; namely carbohydrates, tartrates and oxalates. That is, the said cooling ingredient or ingredients may be introduced in various manners, to suit conditions; as for instance, actual incorporation with the other ingredients or incorporation with only a portion of the other ingredients or included as separate granules but mixed 40 45 with granules of the other ingredients or with the grains of commercial grades of blasting powders, etc.

It should also be expressly understood that the scope of my invention is not limited to 50 any particular physical form of "safety blasting powders." That is, the physical form of said "safety blasting powders" may vary in any manner whatsoever, to suit commercial application; as for instance, granules, pellets, powders, cubes, cylinders, etc.

55 Summarizing, my "safety blasting powders" consist of one or more carbohydrates in any practicable quantity (preferably from 5 to 35%) together with one or more tartrates and oxalates (preferably from 1 to 15%), used in combination or singly with practicable combinations of metallic nitrates, sulphur and materials that are essentially carbon. Other ingredients 60 65 may also be added to the above in minor

quantities and still be within the scope of my invention, such as organic or inorganic compounds, that will absorb heat through the reduction of oxygen or by their volatilization during the decomposition reactions or by their liberation of water or crystallization or combination of such causes.

Typical formulae, by way of examples, are:

|                                                | Per cent. |    |    |    |    | 75  |
|------------------------------------------------|-----------|----|----|----|----|-----|
| Sodium nitrate                                 | 54        | 43 | 47 | 54 | 40 |     |
| Potassium nitrate                              |           | 10 | 8  |    | 16 |     |
| Sugar                                          |           |    | 5  | 18 |    |     |
| Starch                                         | 17        | 13 |    | 23 | 15 |     |
| Sulphur                                        |           | 5  | 5  | 4  | 4  | 80  |
| Charcoal                                       |           | 17 | 15 | 16 | 19 | 16  |
| Lignite                                        |           |    |    |    | 4  |     |
| Sodium potassium tar-<br>trate (Rochelle salt) |           | 7  |    |    | 4  |     |
| Ammonium oxalate                               |           |    | 5  | 3  |    | 585 |

My investigations indicate that I may vary the physical characteristics of my improved "safety blasting powders" through variations of their densities, granulations, physical forms, etc., and produce similar effectiveness to the grades of blasting powders, now in the coal-mines of the United States, with the advantage of being much less apt to cause the very terrible coal-mine disasters that occur when the inflammable gas and dust mixtures, contained therein, are ignited. I may also see fit to add other ingredients to my "safety blasting powders," as hereinbefore defined, in order to produce the most desirable combinations of effectiveness and safety.

If carried into effect, through substitution of the above described "safety blasting powders" for all the present types of so-called blasting powders, used in American coal mines, my invention will cause the improvement, hereinbefore described, of over 70% of all the explosives, used for blasting coal in the United States.

(See United States Bureau of Mines Technical Paper 340—page 9.)

Having described my invention, what I claim is:

1. A composition consisting of one or more metallic nitrates, sulphur and one or more materials that are essentially carbon, the whole constituting a black blasting powder to which combination is added from 5 to 35% of one or more carbohydrates and 1 to 15% of one or more tartrates and oxalates.

2. A composition consisting of one or more metallic nitrates, sulphur and one or more materials that are essentially carbon, the whole constituting a black blasting powder to which combination is added from 5 to 35% starch and sugar and 1 to 15% sodium potassium tartrate and ammonium oxalate.

3. A blasting powder consisting of from 45% to 65% sodium nitrate, from 1 to 15% sulphur and from 10 to 25% charcoal, to which combination is added from 10 to 30% starch and 1 to 10% sodium potassium tartrate.

4. A blasting powder, consisting of 54%

sodium nitrate, 5% sulphur, 17% charcoal, 17% starch, and 7% sodium potassium tartrate.

In testimony whereof he affixes his signature.

10

CARL D. PRATT.